

1

3,814,794

## THERMAL PROCESS FOR REMOVING SOLVENT FROM POLYBENZIMIDAZOLE CONTINUOUS FILAMENTARY MATERIALS

Arthur E. Prince, Jr., Basking Ridge, N.J., assignor to Celanese Corporation, New York, N.Y.

No Drawing. Filed Mar. 31, 1972, Ser. No. 240,228

Int. Cl. D01d 5/12

U.S. Cl. 264—210 F

7 Claims

## ABSTRACT OF THE DISCLOSURE

An improvement in the process for the removal of solvent from solvent-containing fibrous materials such as dry-spun polybenzimidazole continuous filamentary material is disclosed. The as-spun continuous filamentary material is heated to substantially remove the solvent contained therein without substantial oxidative degradation of the material.

## BACKGROUND OF THE INVENTION

The preparation of polybenzimidazole continuous filamentary materials (e.g., monofilaments and multifilament yarn, strand, cable, tow, etc.) is well known in the art. Generally, a polybenzimidazole is dissolved in a suitable solvent and the solution treated, as by spinning, to produce the continuous filamentary material. The as-spun continuous filamentary materials often contain substantial amounts of residual spinning solvent therein. Such high amounts of contained residual spinning solvent are generally detrimental to the physical properties of the material.

The solvent-containing as-spun material, for example, has relatively low tensile strength. Other physical properties such as initial modulus, etc., also are generally poor.

The presence of residual solvent is also detrimental to the successful performance of other steps often applied to as-spun materials. For example, drawing of the polybenzimidazole continuous filamentary materials is a well-known method for increasing the tensile properties, and particularly tenacity, of the materials. It has been found, however, that polybenzimidazole continuous filamentary materials often explode during a drawing operation resulting in a porous product having relatively low tensile properties.

The explosion problem is believed due in large part to the presence of moisture such as residual spinning solvent in the polybenzimidazole continuous filamentary materials. Residual solvent will also plasticize the fiber during the drawing operation preventing adequate orientation and attainment of target properties. Much attention has therefore been directed to the removal of the solvent from the formed continuous filamentary material. Solvent removal has heretofore been accomplished by washing with a solvent-miscible liquid. The washing step, however, essentially replaces one liquid with another. The presence of any residual washing liquid is also detrimental in drawing. The washed continuous filamentary materials therefore have to be subjected to extensive treatments to remove the wash liquid prior to drawing. These treatments are difficult and expensive. For example, U.S. Pat. No. 3,584,104 discloses washing as-spun polybenzimidazole fiber until it contains less than one percent by weight of the solvent and preferably until the material is essentially free of the solvent. Water is typically used as the wash liquid although other wash materials such as acetone, methanol, methyl ethyl ketone and the like are disclosed to be useful. The washing operation can be conducted by winding the polybenzimidazole continuous filamentary material on perforated rollers or bobbins, immersing the wound bobbins in the liquid wash water

2

and pressure washing the fiber for about 2 to 100 hours or more. Pressure washing is accomplished by passing the wash medium into the interior of the hollow, perforated bobbin and outwardly through the perforations so that the solvent is flushed from the polybenzimidazole material wound thereon. The washed material must then be dried to remove the wash liquid to avoid the explosion problem as noted above.

The solvent-wash procedure is an expensive and time consuming operation requiring time to wind the bobbins, wash time (2 to 100 hours or more) and also time to dry the washed material of the wash liquid.

It is an object of this invention to provide a process for treating as-spun polybenzimidazole continuous filamentary materials to substantially remove residual spinning solvent, which process does not require a washing step.

It is an object of this invention to provide a process for treating as-spun polybenzimidazole continuous filamentary materials without substantial oxidative degradation of the materials.

It is an object of this invention to enhance the physical properties of as-spun polybenzimidazole filamentary material at a relatively low cost and in a relatively short time.

It is also an object of this invention to provide a continuous method for treating as-spun polybenzimidazole continuous filamentary material to substantially remove residual spinning solvent.

## SUMMARY OF THE INVENTION

These and other objects of the invention are provided by a process for removing residual spinning solvent from a spun polybenzimidazole continuous filamentary material containing from about 5 to about 25 percent by weight of residual solvent comprising:

- (a) continuously introducing a continuous length of said residual solvent-containing polybenzimidazole continuous filamentary material into a heating zone at a temperature of from about 200 to about 400°C.;
- (b) continuously passing said continuous length of said polybenzimidazole continuous filamentary material under constant tension through said heating zone for a residence time of from about 5 to about 90 minutes; and
- (c) continuously withdrawing said resulting continuous length of polybenzimidazole continuous filamentary material from said heating zone having a substantially reduced residual solvent content.

## DESCRIPTION OF PREFERRED EMBODIMENTS

## The starting polymer

Polybenzimidazoles are a known class of heterocyclic polymers which consist essentially of recurring units of the following formulas I and II. Formula I is:



wherein R is a tetravalent aromatic nucleus, with the nitrogen atoms forming the benzimidazole rings being paired upon adjacent carbon atoms, i.e., ortho carbon atoms, of the aromatic nucleus, and R' is a member of the class consisting of an aliphatic (alkylene) group, a cycloaliphatic ring, an aromatic ring and a heterocyclic ring such as pyridine, pyrazine, furan, quinoline, thiophene, and pyran.

Formula II is:



wherein Z is an aromatic nucleus having the nitrogen atoms forming the benzimidazole ring paired upon adjacent carbon atoms of the aromatic nucleus.

Preferably, the continuous filamentary materials are prepared from aromatic polybenzimidazoles, that is, from polymers consisting essentially of the recurring units of Formula II and of Formula I wherein R' is an aromatic ring or a heterocyclic ring.

As set forth in the U.S. Pat. 3,174,947 and Reissue Pat. 26,065, which are incorporated herein by reference, the aromatic polybenzimidazoles having the recurring units of Formula II may be prepared by self-condensing a trifunctional aromatic compound containing only a single set of ortho disposed diamino substituents and an aromatic, preferably phenyl, carboxylate ester substituent. Exemplary of polymers of this type is poly-2, 5(6)-benzimidazole prepared by the auto-condensation of phenyl-3,4-diaminobenzoate.

As also set forth in the above-mentioned patents, the aromatic polybenzimidazoles having the recurring units of Formula I may be prepared by condensing an aromatic tetraamine compound containing a pair of orthodiamino substituents on the aromatic nucleus with a dicarboxyl compound selected from the class consisting of (a) the diphenyl ester of an aromatic dicarboxylic acid, (b) the diphenyl ester of a heterocyclic dicarboxylic acid wherein the carboxyl groups are substituents upon carbon in a ring compound selected from the class consisting of pyridine, pyrazine, furan, quinoline, thiophene and pyran and (c) an anhydride of an aromatic dicarboxylic acid.

Examples of aromatic polybenzimidazoles which have the recurring structure of Formula I and which may be formed into fibers or yarns include:

poly-2,2'-(m-phenylene)-5,5'-bibenzimidazole;  
 poly-2,2'-(pyridylene-3",5")-5,5'-bibenzimidazole;  
 poly-2,2'-(furylene-2",5")-5,5'-bibenzimidazole;  
 poly-2,2'-(naphthalene-1",6")-5,5'-bibenzimidazole;  
 poly-2,2'-(biphenylene-4",4")-5,5'-bibenzimidazole;  
 poly-2,2'-amylene-5,5'-bibenzimidazole;  
 poly-2,2'-octamethylene-5,5'-bibenzimidazole;  
 poly-2,6-(m-phenylene)-dimidobenzene;  
 poly-2,2'-cyclohexenyl-5,5'-bibenzimidazole;  
 poly-2,2'-(m-phenylene)-5,5'-di(benzimidazole) ether;  
 poly-2,2'-(m-phenylene)-5,5'-di(benzimidazole) sulfide;  
 poly-2,2'-(m-phenylene)-5,5'-di(benzimidazole) sulfone;  
 poly-2,2'-(m-phenylene)-5,5'-di(benzimidazole) methane;  
 poly-2,2'-(m-phenylene)-5',5"-di(benzimidazole)  
 propane-2,2; and  
 poly-2',2'-(m-phenylene)-5',5"-di(benzimidazole)  
 ethylene-1,2

where the double bonds of the ethylene groups are intact in the final polymer.

The preferred aromatic polybenzimidazole fiber or yarn is one prepared from poly-2,2'-(m-phenylene)-5,5'-bibenzimidazole, the recurring unit of which is:



Any polymerization process known to those skilled in the art may be employed to prepare the polybenzimidazole which may then be formed into a continuous filamentary material and subjected to the drying treatment of the present invention. Preferred techniques used to prepare the polybenzimidazole are disclosed in U.S. Pats. 3,509,108 and 3,551,389, both assigned to the assignee of the present invention and both herein incorporated by reference.

With respect to aromatic polybenzimidazoles, preferably equimolar quantities of the monomeric tetraamine and dicarboxyl compound are introduced into a first stage melt polymerization reaction zone and heated therein at a temperature above about 200° C., preferably at least 250° C., and more preferably from about 270 to 300° C. The reaction is conducted in a substantially oxygen-free atmosphere, i.e., below about 20 p.p.m. oxygen and preferably below about 8 p.p.m. oxygen, until a foamed prepolymer is formed. Usually, the first stage reaction is continued until a prepolymer is formed having an inherent viscosity, expressed as deciliters per gram, of at least 0.1, and preferably from about 0.13 to 0.3, the inherent viscosity (I.V.) as used in the present specification and claims being determined from a solution of 0.4 grams of the polymer in 100 ml. of 97 percent H<sub>2</sub>SO<sub>4</sub> at 25° C.

After the conclusion of the first stage reaction, which normally takes at least 0.5 hours, and preferably 1 to 3 hours, the foamed prepolymer is cooled and then powdered or pulverized in any convenient manner. The resulting prepolymer powder is then introduced into a second stage polymerization reaction zone wherein it is heated under substantially oxygen-free conditions, as described above, to yield a polybenzimidazole polymer product, desirably having an I.V., as measured above, of at least 0.6, e.g., 0.80 to 1.1 or more.

The temperature employed in the second stage is at least 250° C., preferably at least 325° C., and more preferably from about 350 to 425° C. The second stage reaction generally takes at least 0.5 hours, and preferably from about 1 to 4 hours or more.

A preferred method of preparing the polybenzimidazole is disclosed in the aforesaid U.S. Pat. 3,509,108. As disclosed therein, aromatic polybenzimidazoles may be prepared by initially reacting the monomer in a melt phase polymerization at a temperature above about 200° C. and a pressure above 50 p.s.i. (e.g., 300 to 600 p.s.i.) and then heating the resulting reaction product in a solid state polymerization at a temperature above about 300° C. (e.g., 350 to 500° C.) to yield the final product.

#### Preparation of the continuous filamentary material

The term "continuous filamentary material" as used herein is intended to include monofilaments and multifilaments such as strand, yarn, cable, tow, and the like.

As is well known, the polybenzimidazoles are generally formed into continuous filamentary materials by solution spinning, that is, by dry or wet spinning a solution of the polymer in an appropriate solvent such as dimethylacetamide, dimethylformamide, dimethylsulfoxide or sulfuric acid (used only in wet spinning) through an opening of predetermined shape into an evaporative atmosphere for the solvent in which most of the solvent is evaporated (dry) or into a coagulation bath (wet), resulting in the polymer having the desired shape.

The polymer solutions may be prepared, for example, by dissolving sufficient polybenzimidazole in the solvent to yield a final solution suitable for extrusion containing from about 10 to 45 percent by weight of polymer, based on the total weight of the solution, preferably from about 20 to 30 percent by weight.

One suitable means for dissolving the polymer in the solvent is by mixing the materials at a temperature above the atmospheric boiling point of the solvent, for example, 25 to 120° C. above such boiling point, and at a pressure of 2 to 1 atmospheres for a period of 1 to 5 hours.

Preferably, the above polymer solutions, after suitable filtration to remove any undissolved portions, are dry spun. For example, the solutions may be extruded through a spinneret into a conventional type downdraft spinning column containing a circulating inert gas such as nitrogen, noble gases, combustion gases or super heated steam. Conveniently, the spinneret face is at a temperature of from about 100 to 170° C., the top of the column from about 120 to 220° C., the middle of the column from about 140° to 250° C.,

and the bottom of the column from about 160° to 320° C. After leaving the spinning column, the continuous filamentary materials are taken up, for example, at a speed in the range of from about 50 to 350 meters per minute. Further details for a method of dry-spinning polybenzimidazole continuous filamentary materials are shown in U.S. Pat. 3,502,756, Bohrer et al., assigned to the same assignee as the present application, and this patent is hereby incorporated by reference.

The above polymer solutions may also be wet-spun. For example, the polybenzimidazole solutions may be extruded into a coagulation bath containing dimethylacetamide.

Other suitable wet-spinning coagulation baths include polyhydroxy aliphatic alcohols having 2 to 3 hydroxy groups and 2 to 6 carbon atoms as disclosed in U.S. Pat. 3,619,453 to Riggs, assigned to the same assignee as the present invention and herein incorporated by reference. Polybenzimidazoles formed by wet-spinning into coagulation baths containing sulfuric acid are not suitable for use in the present invention.

The as-spun polybenzimidazole continuous filamentary materials generally contain from about 5 to about 25 percent by weight of the materials of residual spinning solvent. The solvent or other moisture content of these as-spun materials should be substantially removed to enhance the properties of the as-spun materials. It has been found, for example, that reduction of residual moisture content to a level below about 2.0, preferably below about 0.5, and most preferably below about 0.1, percent by weight of the materials, allows the materials to be drawn without a substantial explosion problem.

A continuous length of the as-spun polybenzimidazole continuous filamentary material may be continuously introduced into an appropriate heating zone, continuously passed therethrough under constant tension and continuously withdrawn therefrom with a substantially reduced residual spinning solvent content. The brief passage through the heating zone results in no substantial degradation of the fibrous material.

The polybenzimidazole continuous filamentary materials may be heated in the heating zone by any suitable heating means. For example, the materials may be continuously passed into a muffle or radiant heat furnace of appropriate length. Also, the continuous filamentary material may be continuously passed into contact with a heated contact surface such as a hot roll, shoe, pin or plate. Combinations of heating means may also be employed in the heating zone. That is, the continuous filamentary material may be continuously passed through a muffle furnace into contact with a hot shoe or vice versa.

As known in the art, polybenzimidazoles oxidize at high temperatures and turn dark. A loss in physical properties may also result from oxidation. It is therefore preferable that the polybenzimidazole continuous filamentary materials be heated in an inert atmosphere to prevent oxidation of the fibers. An air atmosphere may be used. The material, however, may darken slightly when air is used as the heating zone atmosphere.

Steam may also be used as the heating zone inert atmosphere. The polybenzimidazole continuous filamentary material may pick up water during handling and removal of this water during treatment in the heating zone provides a suitable inert atmosphere.

The continuous length of the polybenzimidazole continuous filamentary material is continuously passed through the heating zone at a temperature of from about 200 to about 400, preferably from about 300 to about 350° C., for a residence time of from about 5 to about 90, preferably from about 10 to about 30, minutes to substantially remove the spinning solvent therein without substantial oxidative degradation of the materials.

The polybenzimidazole continuous filamentary material is continuously passed through the heating zone at

an essentially constant length. That is, as known in the art, the material is maintained under a slight tension as it passes through the heating zone. Polybenzimidazole continuous filamentary materials passed into a heating zone as above without being held under sufficient tension to maintain a constant length of material could shrink up to about 13 percent and thus change the properties of the dried material. While an essentially constant length of material is most preferred, a slight amount of shrinkage is more preferable than any amount of stretching.

The dried polybenzimidazole continuous filamentary materials may then be drawn. Since polybenzimidazole materials have a high natural moisture regain level, the dried continuous filamentary materials should be maintained in a dry, preferably inert atmosphere until drawing is completed. The materials can be maintained, for example, in an atmosphere such as air, argon, nitrogen, carbon dioxide, steam, or the like. The atmosphere is also preferably non-oxidizing.

Drawing of the polybenzimidazole continuous filamentary materials may be performed in any suitable manner according to drawing procedures known to those skilled in the art. Particularly preferred drawing techniques are disclosed in U.S. Pat. 3,622,660 of George F. Ecker and Thomas C. Bohrer and U.S. Pat. 3,541,199 of Thomas C. Bohrer and Arnold J. Rosenthal. Both the patents are assigned to the same assignee as the present invention and are herein incorporated by reference. For example, the polybenzimidazole continuous filamentary materials may be drawn at high drawing speeds, that is, the speed of the supply roll may be on the order of 10 to 50 meters per minute or higher. The limiting factor of the drawing speed is the particular design of the drawing apparatus and the elastic properties of the fiber.

The polybenzimidazole continuous filamentary materials may be subjected to a hot drawing treatment in any convenient hot drawing apparatus or zone, for example, by passing the material over a heated surface such as a hot roll, shoe, pin or plate or by passing the material through a radiantly heated zone, such as a muffle furnace.

Preferably, the continuous filamentary material is passed immediately from the drying step into the hot drawing zone in order to minimize exposure of the material to the atmosphere.

Hot drawing is suitably conducted at a temperature of above about 350° C. up to about the degradation temperature of the polybenzimidazole continuous filamentary material, preferably from about 375 to 650° C., and more preferably from about 390 to 480° C.

The polybenzimidazole continuous filamentary material may be drawn at any desired draw ratio below that at which they break, typically from above about 1.5:1 to 4.5:1, and preferably from about 2.5:1 to 3.5:1. The hot drawing residence time, i.e., the time during which the material is being heated, is usually from about 0.2 to 50 seconds, preferably 0.5 to 10 seconds, and more preferably 0.5 to 5 seconds. Substantially longer residence times at the elevated drawing temperatures may cause degradation. Other suitable polybenzimidazole drawing techniques will be apparent to those skilled in the art.

The resulting drawn polybenzimidazole continuous filamentary materials of the present invention are characterized by a high degree of thermal stability and show great resistance to degradation by heat, hydrolytic media and oxidizing media. They may be used, for example, in deceleration chutes for aircraft, chutes for re-entry capsules, high temperature dust collector bags, non-flammable clothing and fabrics and in spacesuits and flight clothing.

The invention is additionally illustrated in connection with the following examples which are to be considered illustrative of the present invention. It should be understood, however, that the invention is not limited to the specific details of the examples.

7  
EXAMPLE I

A polybenzimidazole yarn, namely, poly-2,2'-(m-phenylene)-5,5'-bibenzimidazole, is selected as the exemplary polybenzimidazole for use in carrying out the process of this invention.

The polymer is formed into an as-spun yarn in the manner described in the Example I of U.S. Pat. 3,502,756 to Bohrer et al. More particularly, a dope of dimethylacetamide containing 23 percent by weight of the polymer is extruded through a 110-hole jet into a dry spinning chamber containing superheated steam as the evaporative atmosphere. A 300/110 yarn (110 filaments making up a yarn having an overall denier of 300) is formed from the as-spun yarn. The yarn contains about 15 percent by weight of the material of residual dimethylacetamide.

Samples of the 300/110 as-spun yarn are strung up to pass over two hot shoes (10 inches contact length each) and through a series of muffle furnaces at a speed of one meter per minute. The temperature of the shoes is maintained at 275° C. while the furnace temperature is varied between 225 and 300° C. Also, the total muffle furnace length is varied from 20 feet to 36 feet. Samples of the thus-heated yarn are measured to determine the tensile strength, percent elongation and the amount of residual solvent. None of the heated samples show evidence of any substantial oxidative degradation.

Details of the runs made and results obtained are shown below in Table I. The data shows that substantial amounts of residual spinning solvent may be reduced with the process of the present invention.

TABLE I

| Sample | Shoe temperature, °C. | Muffle furnace temperature, °C. | Muffle furnace length, feet | Time of heating, minutes |         | Tensile strength, grams/denier | Percent elongation | Percent residual solvent |
|--------|-----------------------|---------------------------------|-----------------------------|--------------------------|---------|--------------------------------|--------------------|--------------------------|
|        |                       |                                 |                             | Shoe                     | Furnace |                                |                    |                          |
| A----- | 275                   | 250                             | 20                          | 0.6                      | 6.5     | 1.59                           | 61.2               | 4.5                      |
| B----- | 275                   | 300                             | 20                          | 0.6                      | 6.5     | 2.04                           | 66.6               | 3.0                      |
| C----- | 275                   | 225                             | 36                          | 0.6                      | 11.5    | 1.44                           | 70.8               | 7.1                      |
| D----- | 275                   | 250                             | 36                          | 0.6                      | 11.5    | 1.45                           | 79.0               | 6.5                      |

## EXAMPLE II

Samples of the as-spun yarn of Example I are dried by continuously introducing the yarn into a 36-foot furnace having a dry, flowing nitrogen atmosphere and continuously passing the yarn therethrough at a speed of one meter per minute at varying furnace temperatures. The continuously withdrawn yarn has a substantially reduced residual solvent content. Measurements similar to those of Example I are made of the resulting yarns. The results are shown below in Table II. None of the samples appear to have any substantial oxidative degradation.

Yarn samples F, G and H are drawn without a substantial explosion problem utilizing the techniques shown in the Example of the aforesaid U.S. Pat. 3,541,199. That is, the yarn is drawn by passing the yarn over a hot shoe at a draw ratio of 2.0:1 at a drawing supply speed of 50 meters per minute and a temperature of 420° C. The resulting yarn is substantially non-porous and has good physical properties.

TABLE II

| Sample | Furnace temperature, °C. | Furnace length, feet | Time of heating, minutes | Tensile strength, grams/denier | Percent elongation | Percent residual solvent |
|--------|--------------------------|----------------------|--------------------------|--------------------------------|--------------------|--------------------------|
| E----- | 275                      | 36                   | 11.5                     | 1.66                           | 55.9               | 4.3                      |
| F----- | 300                      | 36                   | 11.5                     | 1.89                           | 79.8               | 1.6                      |
| G----- | 325                      | 36                   | 11.5                     | 1.77                           | 56.0               | 1.15                     |
| H----- | 350                      | 36                   | 11.5                     | 1.69                           | 43.7               | 0.39                     |

For comparative purposes, samples of the as-spun yarn are wound on a perforated bobbin and washed by pressure washing in the conventional manner such as described in U.S. Pat. 3,584,104 for about 48 hours. The washed yarn is dried in a muffle oven at 150° C. for 160 minutes. The resulting yarn has a tensile strength of 1.4 grams/denier,

70  
75

an elongation of 75.7 percent and contains less than 0.05 percent residual solvent.

The data in Tables I and II above indicate that the spinning solvent used for forming polybenzimidazole continuous filamentary material may be removed by the direct application of heat without significant oxidative degradation of the materials. The samples of yarns treated by the process of the present invention and particularly as shown in Example II, have physical properties comparable with the sample treated in the conventional manner which takes many days longer. The process of this invention thus offers substantial savings in time and equipment.

## EXAMPLE III

15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
728

said polybenzimidazole continuous filamentary material through said heating zone for a residence time of from about 5 to about 90 minutes, said filamentary material being held under a tension sufficient to maintain an essentially constant length of material as it passes through said heating zone,

(c) continuously withdrawing said resulting continuous length of polybenzimidazole continuous filamentary material from said heating zone having a substantially reduced residual solvent content; and

(d) drawing the resulting filamentary material obtained from said heating zone in a drawing zone at a draw ratio of from about 1.5:1 to 4.5:1 and at a temperature above about 350° C. up to about the degradation temperature of the polybenzimidazole continuous filamentary material for about 0.2 to 50 seconds to yield a drawn polybenzimidazole continuous filamentary material.

2. The process of claim 1 wherein said polybenzimidazole continuous filamentary material withdrawn from said heating zone has a residual moisture content less than about 2 percent by weight.

3. The process of claim 2 wherein the said heating zone is at a temperature of from about 300 to about 350° C. and wherein the said continuous filamentary material has a residence time in the heating zone of from about 10 to about 30 minutes.

4. The process of claim 3 wherein the spinning solvent is dimethylacetamide.

5. The process of claim 3 wherein the spinning solvent is dimethylformamide.

6. A process for enhancing the properties of a dry solution spun polybenzimidazole continuous filamentary material containing from about 5 to about 25 percent by weight of residual spinning solvent which comprises:

(a) continuously introducing, without any prewashing to remove said spinning solvent, a continuous length of said as-spun, residual solvent-containing polybenzimidazole continuous filamentary material into a heating zone at a temperature of from about 200 to about 400° C., passing said continuous length of said polybenzimidazole continuous filamentary material

through said heating zone for a residence time of from about 5 to about 90 minutes, said filamentary material being held under a tension sufficient to maintain an essentially constant length of material as it passes through said heating zone,

(b) continuously withdrawing said resulting continuous length of polybenzimidazole continuous filamentary material from said heating zone having a residual moisture content of less than about 2.0 percent by weight; and

(c) drawing the resulting filamentary material in a drawing zone at a temperature of from about 375 to 650° C. and at a draw ratio of from about 1.5:1 to 4.5:1 for about 0.2 to 50 seconds to yield a drawn polybenzimidazole continuous filamentary material.

7. The process of claim 6 wherein the heating zone is at a temperature of from about 300 to about 350° C., wherein the residence time of the filamentary material in the heating zone is from about 10 to about 30 minutes, and wherein the filamentary material withdrawn from said heating zone has a residual moisture content less than about 0.5 percent by weight.

#### References Cited

##### UNITED STATES PATENTS

|           |         |                  |       |           |
|-----------|---------|------------------|-------|-----------|
| 2,210,161 | 8/1940  | Allen            | ----- | 264—205   |
| 2,433,842 | 1/1948  | Griffin          | ----- | 28—62     |
| 2,692,875 | 10/1954 | Weinstock et al. | ----- | 28—62     |
| 2,811,409 | 10/1957 | Clapp et al.     | ----- | 264—206   |
| 2,975,022 | 3/1961  | Taylor           | ----- | 264—206   |
| 3,523,151 | 8/1970  | Steinberg        | ----- | 264—210 F |
| 3,526,693 | 9/1970  | Rulison et al.   | ----- | 264—210 F |
| 3,584,104 | 6/1971  | Bohrer et al.    | ----- | 264—210 F |
| 3,619,453 | 11/1971 | Richards         | ----- | 264—210 F |
| 3,622,660 | 11/1971 | Ecker et al.     | ----- | 264—290 R |
| 3,657,211 | 4/1972  | Bohrer et al.    | ----- | 264—204   |

JAY H. WOO, Primary Examiner

U.S. Cl. X.R.

34—23; 264—184, 204, 290